

# UNITED STATES PATENT OFFICE.

VICTOR EDOUARD BELLEDIN, OF PARIS, FRANCE.

## MANUFACTURE OF SHEETS OF FLEXIBLE ELASTIC MATERIAL WHICH CANNOT BE READILY PUNCTURED.

SPECIFICATION forming part of Letters Patent No. 707,752, dated August 26, 1902.

Application filed March 20, 1901. Serial No. 52,098. (No specimens.)

*To all whom it may concern:*

Be it known that I, VICTOR EDOUARD BELLEDIN, a citizen of the Republic of France, and a resident of Paris, France, have invented 5 a new and useful Improvement in Processes of Making Sheets of Flexible Elastic Material, which improvement is fully set forth in the following specification.

This invention relates to the manufacture 10 of sheets of flexible elastic material which cannot be readily punctured, and is therefore especially suitable for the protection of the inner tubes of double-tube pneumatic tires.

For this purpose the invention consists of the 15 process herein described of making sheets of flexible elastic material, which comprises the steps of cleaning and dehairing the hide of a suitable animal, immersing said hide in a bath of cold crude petroleum, then immers- 20 ing the same in a bath of a mineral or a fatty oil, permitting the hide to dry, immersing the same in a bath of sodium or potassium silicate, cutting from said hide a sheet of suitable width, curling and curving said sheet, 25 immersing the same in benzin, immersing the same in a bath of chlorid of lime, drying the sheet, and immersing the same in a solution of caoutchouc in benzin.

In carrying out my invention the hide of 30 any horned cattle may be employed. The hide is first washed or otherwise cleaned and dehaired by any suitable well-known process. It is then immersed for from two to twenty-four hours in a bath of cold crude petroleum 35 and then from four to twelve hours in a bath of a suitable mineral or fatty oil. After removal from the latter bath it is permitted to dry—that is to say, the excess of oil is permitted to evaporate from the hide. In case 40 the hide is not sufficiently thick for the purpose in view and it is desired to thicken the same, this step is now accomplished by immersing the hide for about twenty minutes in a bath of potassium silicate or sodium silicate having a strength of about 33° Baumé, 45 and the same is then permitted to dry. The next step, either in case the hide has or has not been subjected to the treatment for thickening, is that of cutting the same into sheets 50 of approximately the width of the tread of the tire to be made, which is accomplished

by suitable knives. Each sheet is then subjected to the action of a convex roller passing longitudinally of the sheet, which action causes the same to curl or curve transversely 55 and longitudinally. After the sheet has been thus rolled it is immersed for from six to twelve hours in a bath of benzin, whereby it is hardened. It is then removed and dipped in a bath of chlorid of lime of from 33° to 60 50° Baumé in order to close the pores and sterilize the hide and is then permitted to dry. When dried it is ready to be applied in the manufacture of the tire.

The tire is composed of three principal 65 parts—an inner air-tight expansible air-tube of the common and well-known construction in double-tube vehicle-tires, commonly termed the "pneumatic" or "inner" tube and formed, preferably, of india-rubber, an 70 outer cover or sheath, known as the "tire-cover" or "outer" tube and commonly formed of canvas or other flexible non-expansible web and india-rubber and being cut open at its inner periphery for receiving the inner tube 75 or pneumatic, together with my improved protecting-sheet, prepared as described.

The protecting-sheet of hide is immersed in a solution of caoutchouc in benzin or bisulfid of carbon. This causes it to adhere to 80 the tire-cover and renders it capable of being vulcanized to the cover.

Having thus described my invention, I claim as new and desire to secure by Letters Patent—

1. The process herein described of making sheets of flexible elastic material, which comprises the steps of cleaning and dehairing the hide of a suitable animal, immersing said hide in a bath of cold crude petroleum, then 90 immersing the same in a bath of mineral or fatty oil, permitting the hide to dry, cutting from said hide a sheet of suitable width, curling and curving said sheet, immersing the same in benzin, immersing the same in a bath 95 of chlorid of lime, drying the sheet, and immersing the same in a solution of caoutchouc in benzin, substantially as set forth.

2. The process herein described of making sheets of flexible elastic material, which comprises the steps of cleaning and dehairing the hide of a suitable animal, immersing said

hide in a bath of cold crude petroleum, then immersing the same in a bath of mineral or fatty oil, permitting the hide to dry, immersing the same in a bath of sodium or potassium silicate, cutting from said hide a sheet of suitable width, curling and curving said sheet, immersing the same in benzin, immersing the same in a bath of chlorid of lime, drying the sheet, immersing the same in a solu-

tion of caoutchouc in benzin, substantially as set forth.

In testimony whereof I have signed this specification in the presence of two subscribing witnesses.

VICTOR EDOUARD BELLEDIN.

Witnesses:

EMILE LEDRET,  
EDWARD P. MACLEAN.